# EUROPEAN PATENT APPLICATION

(11) **EP 1 627 942 A1**
(43) Date of publication of application: **22.02.2006**
(21) Application number: 04019456.5
(22) Date of filing: 17.08.2004
(51) Int. Cl.: D01F 6/62, D03D 15/00

(54) **Superfine polyester fiber containing a dye component and the fabric made therefrom**

(71) Applicant: NAN YA PLASTICS CORPORATION, Taipei (TW)
(72) Inventor: Jen, Zo-Chun, Taipei (TW)
(74) Representative: Helms, Joachim

(57) **Abstract**

A gray dope dyed superfine fibre with neutral colour hue and a fabric made thereof, wherein the mono-filament denier of the gray superfine fibre is of 0.03~0.5 denier, and the fabric formed by the gray superfine fibre may be further deeply dyed to a desired colour during dyeing and finishing stage; particularly, when the fabric after deep dye shall possess not only a desired touch of soft and exquite but also a superior quality of colour fastness to dry crocking over level 4, colour fastness to wet crocking over level 3, colour fastness to light over level 3, colour change of colour fastness to laundering over level 4, and colour fastness to laundering with respect to PET. stain resistance over level 4 and colour fastness to laundering with respect to Nylon over level 3.

## Description

### BACKGROUND OF THE PRESENT INVENTION

### 1. Field of the Present Invention

The invention relates to a gray dope dyed superfine fibre and the fabrics made thereof, particularly the fabric may be further deeply dyed to a desired colours by additional dyeing process during dyeing and finishing stage; and the fabric after deep dyeing shall possess not only better touch of soft and exquisite but also a superior quality of colour fastness to crocking, colour fastness to light and colour fastness to laundering.

### 2. Description of Prior Act

Since the fabrics made of the superfine yarn with mono-filament denier of less than 0.5 denier have good touch of soft and exquisite, these kinds of fabric have been favorably received by the public when they appeared on the market, and have been widely used for clothing material and furniture decorating purpose.

However, owing to the high fineness of the fibre the surface area of the fibre relatively increases that causes the fibre unable to be dyed the deep colour even the amount of dyestuff used in dyeing process reaches saturation condition, or the fibre may have been dyed to deep colour but the colour fastness is poor due to failure of penetration of dyestuff into the fibre structure. Therefore presently in order to obtain better colour fastness, the conventional fabrics made of superfine fibre can only be dyed to the even light colour.

For improving the problem of unable to be dyed to deep colour or the problem of poor colour fastness after the fabric is dyed to the deep colour, and further for meeting the requirement of market, the fibre industry have devoted themselves in the related research work, meanwhile some patents of invention were also disclosed such as the International Publication No. WO 02/088444 A1 which provided a fabric made of a superfine yarn containing dope dyed component to improve the colour fastness to laundering and colour fastness to light of the fabric.

The invention disclosed in International Publication No. WO 02/088444 A1 had disclosed that the dope dyed component such as carbon black, pigment, dyestuff were employed and mixed together in proportion to obtain the desired colour.

However, when the method is employed for production, the inherent drawbacks incurred by the method shall include the colour matching and colour mixing to the dope dyed component is extremely difficult, and if subsequently proceeding to change colour of fabric is necessary it shall be extremely difficult to ensure that no any dope dyed component is left inside the pipe although pipe line cleaning work including to drain off the waste water and flush the pipe has completely finished.

Therefore, the above-mentioned method is unsuitable to mass production and unable to meet the requirement of the market of wide variety colour change of fabric.

### SUMMARY OF THE PRESENT INVENTION

For improving the above-mentioned drawbacks, the invention provides a fabric made of superfine yarn containing gray dope dyed component which may be further deeply dyed to different colours under lower dyestuff concentration through additional dyeing process during dyeing and finishing stage.

The fabric of the invention so obtained has good colour fastness to crocking and colour fastness to light, and has the advantage of reducing the loss caused by spending long period of time to drain off the waste water in case of colour change.

Hence, the major purpose of the invention is to provide a superfine yarn having neutral colour hue containing gray dope dyed component and the fabric made of the superfine yarn which mono-filament denier is within a range of 0.01~0.5 denier.

The another purpose of the invention is to provide a fabric made of the gray superfine yarn of the invention may be further deeply dyed to the desired colours during dyeing and finishing stage through additional dyeing process, and particularly the fabric, after dyeing, shall possess not only a desired touch of soft and exquisite but also a superior colour fastness to crocking, colour fastness to light and colour fastness to laundering.

### DETAILED DESCRITION OF THE PREFERRED EMBODIMENTS

Since gray has a neutral colour hue among the three primary colours of red, yellow and green, and does not lean towards any of the three primary colours, the fabric made of the said superfine yarn containing dope dyed component carries no any other colour hue, it is much easier to do colour match when the fabric is deeply dyed to the desired colour through additional dyeing process during dyeing and finishing stage, and the gray dope dyed component can be formed by pigments or dyestuffs, but the dope dyed component formed by pigments provides better colour fastness when applied on superfine yarn.

As for the percentage by weight of the gray dope dyed component added to the polymer of the present invention, no specific restriction is required but it is better to choose the range from 3~15 % by weight in general. When the amount of the gray dope dyed component added is less than 3 % by weight it is apt to causing colour deviation between spindles due to poor mixing effect with polymer. Whereas if the amount of dope dyed component added exceeds 15 % by weight the spinning property and physical property shall be affected and become poor.

The invention also imposes no specific restriction on the form of and manner for adding the dope dyed component to polymer. Normally the method more popularly used for adding the dope dyed component to polymer is making the dope dyed component into the form of masterbatch, and is fed into melting machine together with polymer by employing dosing unit. The polymer mainly used in the invention is polyester. However, other ingredients such as Titanium dioxide, antibiotics, anti-ultraviolet ray agent or anti-flaming agent can also be added to the polymer to obtain other mechanical properties.

The superfine fibre containing dope dyed component of the invention has mono-filament denier of 0.01~0.5 denier, and preferably of 0.03~0.5 denier. When the mono-filament denier is greater than 0.5 denier, the fabric shall be deeply dyed to obtain deep colour with real good colour fastness without the needed of additional dyeing process by using dope dyed component to improve colour fastness.

However, since the filament is in greater denier the fabric lacks the desired touch of soft and exquisite. Whereas when the mono-filament denier is less than 0.01 denier, the fabric will present the desired touch of soft and exquisite, but due to over-fine fibre more amount of dope dyed component is needed for improving the colour value and colour fastness, and the spinning and physical properties of the filament will become worse that cause the product unable to be accepted by customers.

However, there is no any specific restriction is required on the manufacturing of single filament of the superfine fibre containing gray dope dyed component of the invention having a mono-filament denier of 0.01~0.5 denier. The filament may be made of single polyester by direct spinning method, or may be made of polyester and alkali easy soluble copolymerised polyester by bi-component spinning method to form split type or sea island type superfine compound yarn and than the alkali easy soluble copolymerised polyester is removed by employing the alkali-reduction treatment method to obtain superfine polyester fibre; normally when mono-filament denier is less than 0.25 denier the method of bi-component spinning followed by alkali-reduction treatment is often adopted while taking into consideration the productivity of spinning.

In addition, the form of the gray superfine yarn disclosed by the invention is not restricted by any specific requirement, but may be of the draw textured yarn, or full draw yarn, or air textured yarn; or the superfine yarn may be used to form differential shrinkage gray dope dyed superfine draw textured yarn or to form differential shrinkage gray superfine full draw yarn in combination with the high shrinkage yarn having a shrinkage rate of boiling water higher than 15%. Besides, if dope dyed component is added to the high shrinkage yarn having a shrinkage rate of boiling water higher than 15%, better effect is then obtained.

The manner for carrying out the additional dying process of the fabric made of the gray superfine yarn of the invention is not restricted by any specific requirement. The desired colour hue and value of the fabric shall be obtained simply by adjusting the colour value of the gray dope dyed superfine yarn or by adjusting the colour chroma and value of dyestuff.

Following these procedures, the fabric made of the gray dope dyed yarn of the invention shall have the following properties:

**Table 1**

| Test item | | Test results | Test method |
|---|---|---|---|
| Colour fastness to laundering | Colour change | Over level 4 | AATCC 61-2A-1989 |
| | PET Stain resistance | Over level 4 | AATCC 61-2A-1989 |
| | Nylon Stain resistance | Over level 3 | AATCC 61-2A-1989 |
| Colour fastness to crocking | Colour fastness to dry crocking | Over level 4 | AATCC 8-1988 |
| | Colour fastness to wet crocking | Over level 3 | AATCC 8-1988 |
| Colour fastness to light | | Over level 3 | AATCC 16E-1982 (20 hrs) |

From Table 1 it shows that the fabric made of the gray dope dyed superfine yarn of the invention has a colour change of colour fastness to laundering over level 4, a colour fastness to laundering with respect to PET stain resistance over level 4, and a colour fastness to laundering with respect to Nylon stain resistance over level 3 when tested with method AATCC61-2A-1989; and has a colour fastness to dry crocking over level 4, a colour fastness to wet crocking over level 3 when tested with method AATCC8-1988; as well as a colour fastness to light over level 3 when tested with method 16E -1982 (20 hrs).

### PREFERRED EMBODIMENT OF THE INVENTION

The following practical examples and comparative example were tested with the following respective methods when carrying out the test for colour fastness to laundering, colour fastness to crocking and colour fastness to light:
1. Colour fastness to laundering:
   The test method of AATCC61-2A-1989 was employed to carry out the colour change of colour fastness to laundering, the PET stain resistance and Nylon stain resistance. The greater test data shown in test results represents better colour fastness to laundering.
2. Colour fastness to crocking:
   The test method of AATCCB-1988 was employed to carry out the colour fastness to dry crocking and wet crocking. The greater test data shown in test results represents better colour fastness to crocking.
3. Colour fastness to light :
   The test method of AATC16E-1982 (20 hrs) was employed to carry out colour fastness to light. The greater test data obtained means better colour fastness to light.

### Example 1

The mixture of 5 % by weight of GYAT 0610 gray masterbatch and 95 % by weight of PET polyester granules was used as island component, and the alkali easy soluble copolymerised polyester granules containing polyethylene glycol and sulfoisopathalic acid as sea component to produce gray dope dyed sea island type partially oriented yarn (POY) by means of bi-component spinning method. The proportion of sea to island was 30%:70%, filament winding speed is at 2500 m/s, denier of filament is 320 deniers, number of filament is 40, number of island per filament is 37. Then the sea island type POY and the high shrinkage spin draw yarn (SDY) having a shrinkage of boiling water of 40% and d/f = 30 denier/12 filaments were combined to produce differential shrinkage gray dope dyed superfine draw textured yarn of 180 denier/52 filaments through texturing process.

Then the differential shrinkage gray dope dyed superfine draw textured yarn was knitted into cloth by knitting, and the fabric so obtained was then treated by alkali for weight reduction to dissolve and remove the sea component completely having only the island component and high shrinkage yarn remained. Now the mono-filament denier of the island component is 0.07 dpf.

The fabric, after weight reduction, was tested for colour fastness to laundering, colour fastness to crocking and colour fastness to light directly without further additional dyeing process. The test results are as shown in Table 2.

### Example 2

The weight reduced fabric from example 1 is dyed to red by employing additional dyeing process with dyestuff of Dianix red XF 2% under 130 □.

Then the fabric was tested for colour fastness to laundering, colour fastness to crocking and colour fastness to light, the test results are shown in Table 2.

### Example 3

Dyed the weight reduced fabric from example 1 to yellow by employing additional dyeing process with dyestuff Dianix Flavine XF 2% under 130□.

Then the fabric was tested for colour fastness to laundering, colour fastness to crocking and colour fastness to light. The test results are as shown in Table 2.

### Example 4

Dyed the weight reduced fabric from example 1 to blue by employing additional dyeing process with dyestuff Dianix navy XF 2% under 130□.

Then the fabric was tested for colour fastness to laundering, colour fastness to crocking and colour fastness to light. The test results are as shown in Table 2.

### Comparative example 1

Use PET polyester granules containing 0.4 wt% TiO2 as island component, and alkali easy soluble copolymerised polyester granules containing polyethylene glycol and sulfoisopathalic acid as sea component to produce sea island type POY by employing bi-component spinning method. The proportion of sea to island is 30%:70%, filament winding speed is at 2500 m/s, denier of filament is 320 deniers, number of filament is 40, number of island per filament is 37; Then the sea island type POY and the high shrinkage spin draw yarn having a shrinkage of boiling water of 40% were combined to produce differential shrinkage superfine draw textured yarn of 180 denier/52 filaments through texturing process.

Then the differential superfine draw textured yarn was knitted into cloth through knitting process, and the fabric so obtained was then treated by alkali for weigh reduction to dissolve and remove the sea component completely having only the island component and high shrinkage yarn remained. Now the mono-filament denier of island component is 0.07 dpf.

Then dyed the weight reduced fabric with dyestuff Dianix Black XF 6% under 130□, and tested the fabric for colour fastness to laundering, colour fastness to crocking and colour fastness to light by employing the same method as that employed in the example 1 to 4. The test results are as shown in Table 2.

**Table 2**

| Dyestuff | Colour | Colour fastness to laundering | | | Colour fastness to crocking | | Colour fastness to light |
|---|---|---|---|---|---|---|---|
| | | Colour Change | Stain resistance PET | Stain resistance Nylon | dry | wet | |
| Without Dyestuff (Example 1) | Gray | level 5 | level 5 | level 5 | level 5 | level 5 | level 4 |
| Dianix red XF 2% (Example 2) | Red | level 4 | level 4 | level 3-4 | level 4 | level 3-4 | level 4 |
| Dianix Flavine XF 2% (Example 3) | Yello w | level 4-5 | level 4 | level 4 | level 4 | level 4 | level 4 |
| Dianix navy XF 2% (Example 4) | Blue | level 4-5 | level 4 | level 4 | level 4 | level 4 | level 4 |
| Dianix Black XF 6% (Comparative Example 1) | Black | level 4 | level 3-4 | level 2-3 | level 3-4 | level 2-3 | level 4 |

From Table 2 it shows that the fabric of example 1 containing gray dope dyed component made of superfine yarn through knitting has better color fastness to laundering, colour fastness to crocking and colour fastness to light.

Moreover, the fabric of example 2 through example 4 were dyed to deep colours of red, yellow and blue through additional dyeing process during dyeing and finishing stage, and since the fabric in example 2 to 4 are carried no other colour hue, it is easier for matching the colour so that the colour fastness to laundering, colour fastness to crocking and colour fastness to light of example 2 to 4 are still as better as that shown in Table 2.

However the fabric of comparative example 1 was made of the superfine yarn containing no any gray dope dyed component through knitting which was dyed black during dyeing and finishing stage by employing additional dyeing process. The test results shown in Table 2 shows that the fabric had a relatively poor colour fastness to laundering, colour fastness to crocking and colour fastness to light.

## Claims

1. A gray dope dyed superfine polyester fibre, comprising mono-filament denier of 0.01~0.5 denier and containing gray dope dyed component 3~15 % by weight.

2. The gray dope dyed superfine polyester fibre as defined in claim 1, wherein the mono-filament denier of the gray dope dyed superfine polyester fibre is of 0.03~0.5 denier.

3. The gray dope dyed superfine polyester fibre as defined in claim 1, wherein the mono-filament denier of the gray dope dyed superfine polyester fibre is of 0.07 denier.

4. A gray dope dyed superfine yarn made of any of the gray dope dyed superfine polyester fibre as defined in claim 1 to claim 3, comprising gray dope dyed draw textured yarn, gray dope dyed draw full draw yarn, or gray dope dyed draw air textured yarn.

5. The gray dope dyed superfine yarn as defined in claim 4, which is capably combined with high shrinkage yarn having a shrinkage rate of boiling water higher than 15% to form differential shrinkage gray dope dyed superfine draw textured yarn.

6. The gray dope dyed superfine yarn as defined in claim 4, which is capably combined with high shrinkage yarn having a shrinkage rate of boiling water higher than 15% to form differential shrinkage gray dope dyed superfine full draw yarn.

7. A fabric made of any one of the gray dope dyed superfine yeams as defined in claim 4 to claim 6 by knitting, wherein the fabric comprises gray dope dyed component and has colour change of colour fastness to laundering over level 5, colour fastness to laundering with respect to PET stain resistance over level 5, colour fastness to laundering with respect to Nylon stain resistance over level 3; colour fastness to dry crocking over level 5, colour fastness to wet crocking over level 5 and colour fastness to light over level 4.

8. The fabric as defined in claim 7, wherein the fabric is obtained by dyeing to different colours through additional dyeing process during dyeing and finishing stage having colour change of colour fastness to laundering over level 4, colour fastness to laundering with respect to PET stain resistance over level 4; colour fastness to laundering with respect to Nylon stain resistance over level 3; colour fastness to dry crocking over level 4, colour fastness to wet crocking over level 3 and; colour fastness to light over level 3.
